

Feb. 15, 1949.

B. S. ELLEFSON  
FLUORESCENT PRODUCTS AND METHODS  
OF PREPARATION THEREOF

2,461,726

Filed Dec. 8, 1942

2 Sheets-Sheet 1



Bennett S. Ellefson  
INVENTOR

BY John J. Logan  
ATTORNEY

Feb. 15, 1949.

B. S. ELLEFSON  
FLUORESCENT PRODUCTS AND METHODS  
OF PREPARATION THEREOF

2,461,726

Filed Dec. 8, 1942

2 Sheets-Sheet 2



Fig. 3.

*Bennett S. Ellefson*  
INVENTOR

BY *John J. Hogan*  
ATTORNEY

## UNITED STATES PATENT OFFICE

2,461,726

FLUORESCENT PRODUCTS AND METHODS  
OF PREPARATION THEREOFBennett S. Ellefson, Emporium, Pa., assignor to  
Sylvania Electric Products Inc., Emporium, Pa.,  
a corporation of Massachusetts

Application December 8, 1942, Serial No. 468,202

8 Claims. (Cl. 252—301.6)

1

This invention relates to fluorescent materials which, under predetermined excitation, emit light of a character causing the visual sensation of white.

Heretofore, it has been proposed to produce the visual white effect by forming the fluorescent material from a mixture of phosphors which have complementary hues. However, prior to the present invention, no completely reliable method of control has been proposed for preparing the phosphors with the desired characteristics so that the final product possesses the desired uniformity in producing a standard white visual effect. After considerable study and experimentation, I have found that in arriving at the proper mixing proportions, there are a considerable number of factors which should be taken into account and accurately controlled if the desired uniformity of visual white is to be attained. For example, in determining the optimum mixing ratio of two complementary fluorescent components, the following factors should be carefully considered.

1. The absolute energy conversion of the materials in the visible range.
2. Relative visibility of the visible radiations.
3. The effect of particle sizes on the effective visibility.

Accordingly, it is a principal object of this invention to provide a method of control and preparation of a mixture of phosphors to produce a uniform standard white visual response, substantially independently of certain uncontrollable factors in the materials or in the commercial applications thereof.

Another object is to provide an improved method of preparing two fluorescent materials which will yield a white fluorescent hue when mixed in certain fixed ranges of proportions.

Another object is to provide a method of preparation of fluorescent materials producing a white fluorescent response, whereby uniformity of hue from batch to batch is insured within the limits of hue discrimination of the human eye.

Another object is to provide a white fluorescent material wherein the white response is controlled not only by the mixing ratios of the two fluorescent components, but also in accordance with the ratios of the particle sizes of the said components. While heretofore, it has been suggested to mix complementary fluorescent materials to produce a so-called white hue, these prior suggestions have not taught the necessary ratio factors of particle size which must be considered in arriving at the proper mixing ratio. I have found that the mixing ratio is greatly de-

2

pendent upon a satisfactory ratio of particle sizes in the two components. This is particularly true in the case of fluorescent materials to be excited by cathode-ray bombardment.

5 A further object is to provide a method of preparing the components for a mixture of fluorescent materials so that over large batches the resulting fluorescent hue of the mixture under electron bombardment will lie within the limits 10 corresponding to the visual color of a black body curve at temperatures between 6500° Kelvin and 2848° Kelvin.

A feature of the invention relates to a method of preparing a zinc beryllium silicate whose 15 fluorescent hue coefficients can be shifted so as to represent a point on a straight line on the chromaticity chart which passes through any two arbitrarily chosen points of the black body curve located between those representing the temperatures 20 6400° K. and 2848° K.

Another feature relates to a method of preparation of a zinc sulfide whose fluorescent hue 25 coefficients can be shifted so as to represent a point on a straight line on the chromaticity chart 30 which passes through any two arbitrarily chosen points of the black body curve located between those representing the temperatures 6500° K. and 2848° K.

Another feature relates to a mixture of a zinc 35 beryllium silicate and a zinc sulfide which are prepared so that the fluorescent hue coefficient of the resultant mixture can be chosen at any point between that corresponding to a black body at a temperature between 6500° K. and 2848° K.

40 A further feature relates to a method of preparing a zinc beryllium silicate-zinc sulfide white fluorescent mix whereby variations of the effective luminous efficiency of the components in the mix result in deviations from a standard white (e. g. that corresponding to a black body at 6500° K.) substantially along the curve of visible radiation of a black body at a temperature between 2848° K. and 6500° K.

45 A further feature relates to a method of control in the preparation of a white fluorescent mix so that when the mix is applied to devices such as cathode-ray tubes, fluorescent lamps, etc., which are subjected to the usual heat treatment or baking, the green shift of the white hue is 50 reduced to a minimum.

A still further feature relates to a process of preparation of a white fluorescent mix wherein the final product under electron excitation produces a "tangential white" as herein defined.

55 Other features and advantages not specifically

enumerated will be apparent after a consideration of the following detailed descriptions and the appended claims.

In the drawings, Figures 1, 2 and 3 are standard trichromatic color charts, useful in explaining the invention.

Development of white fluorescing materials has been consistently stimulated during the development of television picture tubes of the cathode-ray type. In these tubes the fluorescence of the material is excited by cathode rays impinging on the fluorescent screen at a velocity corresponding to a voltage difference of several thousand volts. White fluorescing materials are also applied to the walls of mercury vapor discharge lamps in which the fluorescence is excited mostly by the ultra-violet light generated in the mercury vapor discharge.

A preferred fluorescent material which yields good white light emission consists of a mixture of manganese activated zinc beryllium silicate with silver activated zinc sulfide. Such a mixture has been described in my previous application, Serial No. 272,559, filed May 9, 1939, now abandoned. The fluorescent hue of the silicate is yellowish, that of the sulfide is bluish, and the dominating colors of the components are complementary. As usual two colors are called here complementary when they complement each other so as to produce the sensation of white if mixed in the proper intensity proportions.

As is taught in colorimetry, any given color sensation can be reproduced by a superposition of three different fixed color stimuli called primaries which may be chosen arbitrarily within limits. Once these three primaries have been chosen, any given color sensation can be expressed in terms of three coordinates or coefficients which are proportional to the intensities of the three primaries.

These primaries have been standardized by the International Commission on Illumination in such a manner that all colors can be expressed by positive color coordinates (trichromatic coefficients) and the proportionality constant has been so chosen that the sum of the three coordinates of a color is always equal to unity. Accordingly, any color is completely determined by only two of the three coefficients, say by  $x$  and  $y$ ; because the third coefficient ( $z$ ) is fixed by the condition  $x+y+z=1$ . The I. C. I. primaries do not correspond to real colors existing in nature. Their choice was determined by a number of advantages which could not be secured by any set of natural primaries.

These advantages are: First, any hue is completely determined by only two of the three coefficients; second, for a spectral color, one of the coefficients is equal to the visibility of that color, as defined by the sensitivity of the human eye for the different wave lengths of the visible spectrum; third, all real colors can be expressed by positive coordinates smaller than one; furthermore, the standard coordinates are linear functions of other coordinates based on any set of primaries chosen from the range of real colors (within limits).

As a result of this linear relation between the standard primaries and the spectrum colors, the hue resulting from the mixture of two given additive colors has trichromatic coefficients corresponding to a point located on a straight line connecting the two points representing the component colors. In the standard color charts,  $x$  is the I. C. I. red content,  $y$  is the standard visi-

bility or the I. C. I. green content of any given hue.

A reasonable definition of a white standard in these coordinates would be the point with the coordinates  $x=\frac{1}{3}$ ,  $y=\frac{1}{3}$ . This definition is, however, not practical because it can not be readily reproduced and is decidedly on the purplish side of white. Three reproducible white light sources have, therefore, been chosen as standards of illumination for color matching. These three white standards are called, respectively, Illuminant A, Illuminant B and Illuminant C. Illuminant A corresponds very nearly to the color of a black body at a temperature of 2848° Kelvin. Illuminant B corresponds to the color of a black body at 4800° Kelvin. Illuminant C to that of a black body at 6500°. Illuminant C is very nearly the color of average daylight and is, in this sense, a reasonably absolute white standard.

Standards A and B are white in a psychological sense because they are in a region of certain artificial light sources which have been used for centuries. For further details of the standard chromaticity coefficients and their calculations from color measurements made with standard color filters, see Hardy's Handbook of Colorimetry, MIT press, Cambridge, Massachusetts, 1936.

Usually a curve representing the spectral colors in the  $x-y$  plane is drawn into the standard chromaticity diagram, as shown in Fig. 1. This diagram is drawn to scale and the curve 780-520-410 represents the curve of pure spectral colors whose wavelengths in light wave units ( $\text{mm}\mu$ ) are designated thereon. The blue content of a given point in this chart is only given by implication; as the primary blue content of a hue is represented by its  $z$  coordinate. The curve representing the spectrum colors makes it possible to recognize the "blue," "green" and "red" regions in the  $x-y$  plane. Charts of this kind into which the curve for the spectrum colors are printed and their wave lengths marked, can be bought on the market. They are practically indispensable for a convenient graphical representation of color data.

As has been mentioned before, the I. C. I. chromaticity coordinates are so chosen that the mixture of any two additive colors picked at random produce a sensation which corresponds to a point on the straight line connecting the two points representing the arbitrary picked colors in the  $x-y$  plane of the chromaticity chart.

Referring to Fig. 1, let one of the components 55 of the fluorescent material be so chosen with a color on the blue side of point C, say at C' on line CB, the other with a color on the yellow side of point B, say B' on line BC. The line CB intersects the spectral curve at the red end at approximately 577.7  $\text{mm}\mu$ . This line also intersects the spectral curve at the blue end at approximately 477.8  $\text{mm}\mu$ . The line which is tangent at point A intersecting the black body curve at A and a point immediately adjacent thereto 60 lying between A and B intersects the spectral curve at approximately 586  $\text{mm}\mu$ , and at the blue end at approximately 490  $\text{mm}\mu$ . The resulting sensation of two stimuli having the coordinates C' and B' will be located on the line connecting the points B' and C'. The exact location of the resulting sensation on line B' and C' depends on the mixing ratio of the two components. To give a concrete example, assume that a 50-50 mixture produces a sensation corresponding to a point exactly half way between points B and

C, then the addition of a small quantity of component C' will shift the hue of the mixture a little toward the point C. Inversely, a small excess of B' will shift the coordinates of the resulting sensation toward point B. Any variation of the original ratio will, therefore, shift the coordinates of the resulting sensation from one standard white, say C, to another standard white, say B, substantially along the curve of black body radiation.

I have found that the processing of two components of a fluorescent mixture can be carried out in such a way that their respective fluorescent hues are represented by two points located on a line passing through the I. C. I. standard white points B and C. This objective can be attained in accordance with the following disclosures.

The coordinates of the silicate component can be shifted between the yellowish and greenish regions by varying the ratio of zinc to beryllium, and by varying the firing time and the activator concentration. The fluorescent hue of the sulfide component, on the other hand, may be shifted back and forth between the bluish and greenish region by the proper choice of activators and their concentration and of firing time and temperature. The paths of the chromaticity points of the two components obtained by these processing variations are substantially perpendicular to the line BC in the chromaticity chart of Fig. 1. Therefore, by proper processing control the points of intersection of these paths with line BC can be achieved. The processing conditions for the two components which will lead to these intersection points will be described. They will be described and form a part of the invention.

I. The preferred method of making a sulfide component with a fluorescent hue whose representative chromaticity point is located on a straight line connecting points B and C on the I. C. I. chromaticity chart includes the following steps. The zinc sulfide is precipitated with hydrogen sulfide from purified zinc sulfate to which has been added 0.0005% by weight of silver in the form of  $\text{AgNO}_3$ . After drying, 7% sodium chloride by weight is added. The mass is then milled for three hours and fired at  $900^\circ\text{C}$ . for 25 minutes.

It is extremely important that the ingredients are very pure because the energy conversion of the sulfide material under excitation is very sensitive to impurities, in particular against iron and nickel. The sensitivity of the silicate is in this respect not quite as high as that of the sulfide in which a few parts in a million will already reduce the luminescent efficiency very markedly. The sulfide in addition is very sensitive to grinding, i. e., to pressure and shock. Milling above two hours produces a marked loss in efficiency. The silicate is only moderately sensitive against grinding but the grinding time must be kept below 30 hours in the average ball mill in order to avoid a decrease in luminescent efficiency.

II. A corresponding silicate component is obtained as follows.  $\text{ZnO}$ ,  $\text{BeO}$  and  $\text{SiO}_2$  or compounds which decompose into them on subsequent heating are well mixed in such proportions as to yield in the final product 40 mol percent  $\text{ZnO}$ , 23 mol percent  $\text{BeO}$ , 37 mol percent  $\text{SiO}_2$ . To these compounds is added  $\text{MnF}_2$  in a quantity such that in the final luminescent material approximately 1.61% manganese by weight will be present. These raw materials are well mixed

and then melted at a temperature between  $1400^\circ$  and  $1500^\circ\text{C}$ . After cooling, the partly devitrified melt is crushed and then ground by milling in a porcelain ball mill using acetone as a milling vehicle. After the material has been reduced to a fineness of thirty microns or less, the dried material is reheated at  $1000^\circ\text{C}$ . for a period of 45 minutes. The time depends somewhat on the size of the crucible. After this low temperature reheating, the material is again milled in a conventional ball mill for a few hours to break up the sintered particles resulting from the second heat treatment, resulting in a wide range of particle sizes from 100 microns down to 0.1 micron.

While the trichromatic coefficients representing each component can be kept with sufficient accuracy within the limits desired for successful location on the line BC, it is impossible to secure uniform energy conversion from batch to batch. (A possible color shift of the sulfide component due to baking of the material, after application to a glass wall or other support, will be discussed later.) The variation of luminous efficiency is substantially due to two factors. The two components must be mixed for proper distribution of the materials before application to the screen. The mixing operation itself will influence the luminous efficiency of the sulfide due to sensitivity of the sulfide to pressure and shock. So high is the sensitivity of the sulfide in this respect that an undesirable variation in luminous efficiency of this component can hardly be avoided.

The sulfide component and the silicate component are basically different materials, and their surface properties, such as encountered in colloids, are for this reason considerably different. Surface properties that determine dispersion conditions in a liquid are, in addition, very susceptible to extremely small variations in processing conditions. These variations in surface properties and the corresponding variation in dispersability are significant in screen application methods in which preferential settling from a suspension containing two components is a factor in changing the ratio of components actually reaching the surface to be screened. This variation in actual ratio would also act in a manner similar to diminution or reenforcement of energy conversion ability of one of the components in its effect on the color of the combination, although the total brightness would not necessarily be affected in the same manner.

Another factor which enters into reproducibility of color is the effective ratio of components. This is due to variations in particle size of the milled silicate component even under reasonably well controlled conditions of milling. A given weight ratio of components would not consistently produce matched surface ratios exposed to the electron beam excitation under these conditions.

The chart which carries the standard trichromatic diagram also carries the curve of black body radiation (dot-dash curve). Three luminous black body conditions are identified in the drawing by the temperatures  $2848^\circ\text{K}$ ,  $4800^\circ\text{K}$ , and  $6500^\circ\text{K}$  respectively at points A, B and C. As can be seen from inspection of Fig. 1, the curvature of the black body curve between points C and B of the I. C. I. color chart is very slight, and a shift of a point from B to C along the straight line BC is for all practical purposes identical with a shift from B to C along the black body curve. The white fluorescence resulting

from the mixture of components according to the invention is therefore identified herein as "tangential white."

A preferred tangential white fluorescent mixture is obtained by mixing, in a ratio between 1 to 2.88, and 1 to 3.12, the sulfide designated by I with the silicate designated as II.

In addition to this preferred tangential white mixture, other tangential whites may be obtained by mixing blue sulfides and yellow silicates, which produce fluorescent hues located on other straight lines passing through two neighbouring points of the black body curve within the range of the standard illuminants A, B and C. An example is the location of the chromatic representative points of the components of the mixture on line AB (Fig. 2), which may be considered as a tolerance line for a tangent drawn through a point T of the black body curve as shown in Fig. 3. The tolerance is justified by the fact that the human eye does not discriminate more than about 160 different color shades, and a slight deviation of a hue above or below the black body curve is, therefore, not noticeable if limited to a reasonable value.

In contrast to these tangential whites, "intersecting" whites may be produced by mixing components of a fluorescent material which have dominant spectrum colors located on any of the straight lines corresponding to selected pairs of complementary colors, twelve of which have been defined by Sinden in 1923. Review of Scientific Instruments, volume 11, pages 1123-1153, published by the American Institute of Physics, New York, New York. In particular, Sinden's pair No. 2, which gives theoretically the maximum relative energy efficiency, is such an "intersecting" white. The corresponding straight line passing through line B has been drawn into Figs. 1, 2 and 3, as well as the line corresponding to Sinden's complementary pair No. 12, which yields also an "intersecting" white.

I have found that the cooperating component fluorescent materials with hues located on the line marked "Sinden -2-" on the chromaticity chart may be obtained by mixing sulfide VII with

2 are more critical, and result in more noticeable deviations from desirable white hues, than mixture I plus II, which has been discussed above BC white, or the mixtures III plus IV, or of I with either IVa, V, or VI of the processing table given hereinbelow. As a result, uncontrolled variations of the effective luminous efficiency of the components of a white fluorescent mixture result substantially in a deviation from any of the white points between A and C originally chosen as standard to another point of the black body curve also located between A and C.

According to the status of the art, it is assumed that the choice of the component materials for a white mixture is not critical as long as they are chosen in pairs so as to represent complementary colors in the range between Sinden 1 and Sinden 12. What I believe is new in my finding above the prior art, may be summarized as follows.

1. It is not essential to select the pairs of component materials so that their respective hues are complimentary in the sense defined by Sinden, i.e. with respect to point B.

2. The range of complementary pairs is critical, and must be chosen so as to conform with the rules of a "tangential white" as defined herein.

The following table gives an outline of some of the processing methods which yield components for various white mixtures according to the invention.

The numerical influence of the increase of BeO, activator percentage and devitrification period of the hue shifting of the silicate component toward longer wave lengths is clearly indicated in the table.

Similarly, the table gives a numerical guide for the shifting of the hue of the sulfide component toward shorter wave lengths with increase of the silver activator percentage. A shifting of the hue of the sulfide component fluorescence toward longer wave lengths as indicated in the table, can be obtained by adding a copper activator, which, as is well known, will also increase the period of phosphorescence of the sulfide.

#### Processing table

|      |                                                |                                                      |                                                                                              |
|------|------------------------------------------------|------------------------------------------------------|----------------------------------------------------------------------------------------------|
| III  | Zn Sulfide<br>(0.003% Ag plus)<br>(0.0005% Cu) |                                                      | Fired at 900° C. for 25 minutes, particle size 0.1 to 1.0 micron.                            |
| IV   | ZnBe Silicate<br>(0.50% Mn)                    | ZnO 43 mol per cent<br>BeO 20<br>SiO <sub>2</sub> 37 | Melted at 1400° to 1500° C. Devitrified at 1000° C., 1-4 hours.                              |
| IVa  | ZnBe Silicate<br>(2% Mn)                       | ZnO 40 mol per cent<br>BeO 23<br>SiO <sub>2</sub> 37 | Melted at 1400° to 1500° C. Devitrified at 1000° C., for 1-4 hours.                          |
| V    | ZnBe Silicate<br>(1% Mn)                       | ZnO 37 mol per cent<br>BeO 27<br>SiO <sub>2</sub> 36 | Solid phase reaction 1280° C. for 2-6 hours, particle size selected 6 microns to 0.1 micron. |
| VI   | ZnBe Silicate<br>(1% Mn)                       | ZnO 37 mol per cent<br>BeO 27<br>SiO <sub>2</sub> 36 | Particle size, 15 microns to 0.1 micron.                                                     |
| VII  | Zn Sulfide<br>(0.005% Ag)                      |                                                      | Fired at 900° C. for 25 minutes, particle size 0.1 to 1.0 micron.                            |
| VIII | ZnBe Silicate<br>(1% Mn)                       | ZnO 49 mol per cent<br>BeO 15<br>SiO <sub>2</sub> 36 | Solid phase reaction 1280° C. for 2-6 hours, particle sizes 3 microns to 0.1 micron.         |
| IX   | ZnBe Silicate<br>(1% Mn)                       | ZnO 49 mol per cent<br>BeO 15<br>SiO <sub>2</sub> 36 | Solid phase reaction 1280° C. for 2-6 hours, particle sizes 6 microns to 0.1 micron.         |

either of the silicates VIII or IX processed as indicated in the processing tables given hereinbelow. I have also found, that mixtures made from cooperating components following Sinden's

To produce "tangential white" the preferred mixing ratio of sulfide I (column 5 supra) with silicate II (columns 5 and 6 supra) or one of the silicates IVa to VI is between the limits 1:2 and

1:3, for sulfide III and silicate IV the preferred mixing ratio is 1:3.

The preferred mixing ratio of sulfide VII with silicates VIII or IX is 1:1 which however does not produce a "tangential white."

In the processing of cathode ray tubes, discharge lamps and such electronic devices, it is necessary to bake the tubes during the exhausting process in order to remove adsorbed or absorbed gases which might later be given off and affect the life of the tubes. It is desirable to bake at the maximum temperature which is determined either by the material of the envelope or by the component parts of the tube in order to accelerate the removal of gas. In a device in which fluorescent zinc sulfide is one of the component parts, the zinc sulfide becomes the limiting factor for the baking temperature. At a temperature of 350° C.—375° C., the fluorescent zinc sulfide undergoes a gradual but permanent shift in dominant fluorescent color from blue to blue-green. The effect of baking on a composite mixture, employing a stable yellow fluorescent color complementary to the original blue of the sulfide, is, therefore, a slight shift from the original white in the greenish direction. When the original spectrum colors of the two components are chosen so that they fall approximately on a line going through points B and C, this effect is very much reduced.

This is partly due to the fact that the shift of the blue sulfide component towards the greenish side as a result of baking during exhaust is less pronounced if the sulfide has been so processed that its dominant pre-exhaust hue does not correspond to the very short (blue) frequencies of the spectrum colors characteristic of the sulfide component needed for the subsequent maximum white efficiency of the mixture of silicate with sulfide. As far as I am aware, this feature has not been disclosed heretofore though it is of great practical importance in the manufacture of commercial devices such as cathode-ray tubes, fluorescent lamps, etc.

While in the foregoing disclosure reference has been made to mixtures of fluorescent materials which are composed of sulfides and silicates whose visual hues mix in an additive relation, it is understood that the scope of the invention includes also the application of the "tangential white" principle employing components in which the radiation produced by one of these components is partly absorbed by the other component, or where each component partly absorbs the radiation emitted by the other. Also the invention includes within its scope the use of mixes of the "tangential white" character in which the radiation emitted by one of the components stimulates visible fluorescence or phosphorescence in the other component.

Various changes and modifications may be made herein without departing from the spirit and scope of the invention.

This application is a continuation-in-part of application Serial No. 272,559, filed May 9, 1939 (now abandoned).

What I claim is:

1. The method of producing a fluorescent white mixture with substantially uniform reproducibility of fluorescent white color in accordance with a trichromatic coefficient chart of the type illustrated in the accompanying drawing on which is plotted the curve of black body radiation between 2848° K. and 6500° K., which comprises selecting two fluorescent phosphors

of substantially complementary fluorescent colors, the respective trichromatic coefficient points of which on said chart define a straight line which is substantially tangent to the said black body curve at any point between 2848° K. and 6500° K., the limits of the complementary dominant wavelengths at the red end of the spectrum being between 577.7 mm $\mu$  and 586 mm $\mu$  and the limits of the said complementary dominant wave-lengths at the blue end of the spectrum being between 477.8 mm $\mu$  and 490 mm $\mu$  and mixing said two phosphors to produce a resultant fluorescent color having trichromatic coefficients corresponding to said point of tangency.

2. The method of producing a fluorescent white mixture with substantially uniform reproducibility of fluorescent white color in accordance with a trichromatic coefficient chart such as illustrated in the accompanying drawing and on which is plotted the curve of black body radiation between 2848° K. and 6500° K., which includes the steps of selecting two fluorescent phosphors of substantially complementary fluorescent colors, the respective trichromatic coefficient points of which on said chart define a selected straight line which is tangential to said black body curve at the point whose trichromatic coefficient determines the desired color to be produced, the limits of the spectral colors of said materials at the blue end of the spectrum being determined by the intersection with the spectral color curve on said chart of a first straight line tangent to the black body curve at point 2848° K. and by another straight line which intersects said spectral color curve and which is tangent to said black body curve at the point 6500° K., and mixing the phosphors in a ratio determined by the distance of their respective trichromatic coefficient points from said point of tangency on said selected straight line.

3. The method of producing a fluorescent white mixture with substantially uniform reproducibility of fluorescent white color in accordance with a trichromatic coefficient chart such as illustrated in the accompanying drawing and on which is plotted the curve of black body radiation between 2848° K. and 6500° K., which includes the steps of selecting a bluish fluorescent phosphor having a spectral color at the blue end of the spectrum whose limits are defined by the intersection of two straight lines with the spectral color curve on said chart, one of said lines being tangential to the black body curve at the point 2848° K. and the other line being tangential to the black body curve at the point 6500° K.; selecting a yellowish fluorescent phosphor having a spectral color whose limits are defined by two straight lines, one of which is tangential to the black body curve at 6500° K., and the other of which is tangent to the black body curve at 2848° K.; selecting any desired straight line which is tangential to said black body curve between said points 2848° K. and 6500° K., and whose points of intersection with said spectral color curve are located between the aforementioned limits, selecting a first point on said selected line to one side of its point of tangency with the black body curve, selecting a second point on said selected line on the opposite side of said tangency point, and mixing said two phosphor powders in accordance with the distance between each of said first and second points with respect to said point of tangency to produce a resultant mixture whose resultant fluorescent color has trichromatic coefficients corresponding to said point of tangency.

## 11

4. The method according to claim 1 in which manganese-activated zinc beryllium silicate and silver-activated zinc sulfide are selected as the phosphors, the zinc beryllium silicate having an excess of silica, the molar percent ZnO to BeO being between 1.37 to 1 and 3.26 to 1, said phosphors having a particle size of between 0.15 and 0.1 microns, the sulfide having been fired at approximately 900° C. and the silicate having been melted at a temperature between 1400° C. and 1500° C., and devitrified approximately 1000° C., and the said powders being mixed in a ratio between and including 1:2 and 1:3.

5. The method according to claim 4 in which the silicate powder is chosen with a 37 mol. % ZnO, 27 mol. % BeO, and 36 mol. % SiO<sub>2</sub>.

6. The method according to claim 4 in which the zinc beryllium silicate is prepared so as to contain 43 mol. % ZnO, 20 mol. % BeO, and 37 mol. % SiO<sub>2</sub>.

7. The method according to claim 4 in which the zinc beryllium silicate is prepared so as to contain 49 mol. % ZnO, 15 mol. % BeO, and 36 mol. % SiO<sub>2</sub>.

8. The method according to claim 1 in which one of the phosphors is prepared as a silver-acti-

10

vated sulfide containing 0.0005% silver by heating it at approximately 900° for about 25 minutes, the other phosphor being prepared as a manganese-activated beryllium zinc silicate containing

5 37 mol. % ZnO, 27 mol. % BeO, and 36 mol. % SiO<sub>2</sub>, which is heated from 2 to 6 hours at approximately 1200° C.; and the two phosphors are mixed in a ratio of from 1:2 to 1:3.

BENNETT S. ELLEFSON.

12

## REFERENCES CITED

The following references are of record in the file of this patent:

## UNITED STATES PATENTS

|    | Number     | Name      | Date          |
|----|------------|-----------|---------------|
| 15 | Re. 12,812 | Hammer    | June 16, 1908 |
|    | 907,598    | Hewitt    | Dec. 22, 1908 |
|    | 2,118,091  | Leverenz  | May 24, 1938  |
| 20 | 2,171,145  | Leverenz  | Aug. 29, 1939 |
|    | 2,219,929  | Kaufmann  | Oct. 29, 1940 |
|    | 2,243,097  | Henderson | May 27, 1941  |

## FOREIGN PATENTS

|    | Number  | Country       | Date          |
|----|---------|---------------|---------------|
| 25 | 480,356 | Great Britain | Feb. 22, 1938 |